

## [54] ELECTRIC CONDUCTIVE CERAMIC GUIDE

[75] Inventor: Ryoso Matsumoto, Kyoto, Japan

[73] Assignee: Oda Gosen Kogyo Kabushiki Kaisha, Komatsu-shi, Ishikawa-ken, Japan

[22] Filed: Jan. 8, 1973

[21] Appl. No.: 321,979

## [30] Foreign Application Priority Data

July 7, 1972 Japan..... 47-67569

[52] U.S. Cl. .... 226/196

[51] Int. Cl. .... B65h 23/04

[58] Field of Search .... 226/196, 197, 198, 199; 242/76

## [56] References Cited

## UNITED STATES PATENTS

|           |         |                |           |
|-----------|---------|----------------|-----------|
| 3,143,270 | 8/1964  | Cohen.....     | 226/196   |
| 3,087,665 | 4/1963  | Thomas .....   | 226/198 X |
| 2,862,715 | 12/1958 | McDonald ..... | 226/196   |

Primary Examiner—Allen N. Knowles

Assistant Examiner—Gene A. Church

Attorney, Agent, or Firm—Cushman, Darby &amp; Cushman

## [57] ABSTRACT

An electro-conductive ceramic guide made by the use of a mixture of a metallic titanium and metallic titanium dioxide prepared at a mol ratio of 1 : 0.06 – 1.22, molding this mixture into an element of desired shape, and sintering the shaped element at 1,200° – 1,450° C in vacuum or in an inert atmosphere to cause the crystal particles of the element to have a face-centered cubic crystal structure. The resulting element is mounted at a site where it is brought into a running tape or like article. This guide is of a very small friction coefficient and imparts a stable low tension to the running tape, and has a high electro-conductivity thereby being capable of removing static charge of the tape and is highly suitable for guiding video tapes and computer tapes.

3 Claims, 5 Drawing Figures



PATENTED MAR 26 1974

3,799,422

SHEET 1 OF 2

FIG. 1



FIG. 2



FIG. 3



PATENTED MAR 26 1974

3,799,422

SHEET 2 OF 2

FIG. 4



FIG. 5



## ELECTRIC CONDUCTIVE CERAMIC GUIDE

### BACKGROUND OF THE INVENTION

#### 1. Field of the Invention

The present invention is concerned with a guide for the tapes used in electromagnetic tape recorders, video-tape recorders and electronic computers and for guidance of filaments or films required in the manufacturing process of man-made fibers or films, and also is concerned with the manufacturing method of such guide.

#### 2. Description of the Prior Art

In general, there have been used metal guides for the tapes in electro-magnetic tape recorders, video-recorders and electronic computers. In these metal guides, it has been the practice to give the metal guide an appropriate smoothness to its surface by applying hard chrome-plating onto the surface of the metal guide in order to reduce the friction resistance produced at the time the metal guide is brought into contact with the running tape and in order to impart a stable tension to the running tape.

However, such a conventional metal guide tends to produce uneven surface wear due to the friction occurring during the contact between the metal guide and the running tape during use, resulting in changes in the friction coefficient, and this in turn gives rise to uneven tension in the magnetic tape. As a result, there are produced fluctuations in the reproduction signal frequency due to the fluctuations in the speed of the running tape occurring at the time of recording and reproduction, or in other words there develops the so-called "wow-flutter" phenomenon. Thus, the conventional metal guides had the drawback that it was difficult to effect recording and reproduction of sounds and images of highly good quality.

### SUMMARY OF THE INVENTION

It is, therefore, the primary object of the present invention to eliminate the aforesaid drawbacks and inconveniences of the prior art and to provide an improved guide which insures that always a stable tension is applied to the running tape or like article so that it is possible to obtain good recording and reproducing signals during the use of the guide for an extended period of time.

Another object of the present invention is to provide an electro-conductive ceramic guide which produces very little frictional resistance when it is in contact with a running tape or like article.

Still another object of the present invention is to provide an electro-conductive ceramic guide which does not develop uneven surface wear during use, i.e., during its contact with a running tape or like article.

Yet another object of the present invention is to provide a method of manufacturing the guide of the type described above.

### BRIEF DESCRIPTION OF THE DRAWINGS

FIG. 1 is a longitudinal sectional view of the guide representing the first embodiment of the present invention.

FIG. 2 is a longitudinal sectional view of the guide representing the second embodiment of the present invention.

FIG. 3 is a chart showing the relationship between the friction coefficient and the load.

FIG. 4 is a chart showing the relationship between the friction coefficient and the temperature.

FIG. 5 is a chart showing the relationship between the friction coefficient and the relative humidity.

### DETAILED DESCRIPTION OF THE PREFERRED EMBODIMENTS

After an extensive research to obtain recording and reproducing signals of good quality continuously for a lengthy period of time by the constant application of a stable tension to a running tape, it was found that an electroconductive ceramic guide consisting of a shaped sintered element of titanium monoxide whose crystal structure is that of face-centered cubic was outstandingly superior as a guide for magnetic tapes. This discovery has led to the present invention.

Description will hereunder be made on some of the embodiments of the present invention by referring to the accompanying drawings.

FIG. 1 is a longitudinal sectional view of the first embodiment of the guide of the present invention. In FIG. 1, reference numeral 1 represents the body of a guide element A having a hollow cylindrical configuration. 2 represents a metal screw. 3 represents a bottom plate of the guide element. 4 represents a metal base nut. Both the body 1 of the guide element and the bottom plate 3 are formed integrally with a sintered shaped titanium monoxide having crystal particle consisting of face-centered cubic crystal structure. The metal screw 2 passes through the hollow portion of body 1 and the bottom plate 3 and threadably passes through the base nut 4 and engages the support 5 to which the element is to be attached.

FIG. 2 is a longitudinal section view of the second embodiment of the guide of the present invention. In FIG. 2, reference numeral 6 represents the body of a guide element B of a hollow tapered cylindrical configuration. 7 represents a threaded rod having male threaded portions formed at the opposite ends. 8 represents a top plate of element B. 9 represents a bottom of the plate of the element B. These plates are integral with the body 6. 10 represents a metal top-nut. 11 represents a metal base-nut. The body of the guide element B, the top plate 8 and the bottom plate 9 of the guide element B are each formed with a shaped sintered titanium monoxide having crystal particles consisting of face-centered cubic crystal structure. Also, the threaded rod 7 passes through the hollow portions of the bottom plate 9, the body 6 and the top plate 8 and threadably engages the top-nut 10 at the upper end and threadably engages the base-nut 11 at the lower end, and therefrom threadably engages the support 12 to which the element is to be attached.

Next, description will be made on an example of the method of manufacturing the guide of the present invention.

Metallic titanium powder and metallic titanium oxide which are the starting materials are mixed together at a mol ratio of 1 : 1 and the resulting mixture is shaped into a desired configuration by compression molding. This shaped mixture is sintered in an inert gas (such as argon) at 1,300°C. As a result, there is obtained a sintered, very hard and firm element including the bottom and/or the top plates. Moreover, this sintered element consists of a sintered and molded titanium monoxide whose crystal particles are of face-centered cubic crystal structure. Accordingly, it is only necessary to make

the body 1, the bottom plate 3 of the guide element A of the first embodiment, the body 6, the top plate 8 and the bottom plate 9 of the guide element B of the second embodiment in accordance with the example of the method stated above. It should be noted that it is never harmful to add about 1 percent of powder of clay or the like to the mixed starting materials in order to elevate the effect of sintering.

The guide element A or B of the first or the second embodiment which is obtained in this way is of portions serving as a guide which are brought into contact with a running tape-like article, so that this guide A or B is capable of continuously imparting a very stable tension to the tape-like article, particularly a magnetic tape.

According to the experiment conducted by the inventor, the electro-conductive ceramic guides each consisting of a sintered  $TiO$  and being a shaped sintered titanium monoxide element whose crystal particles had a face-centered cubic crystal structure, i.e., the electro-conductive ceramic guides consisting of sintered materials having  $TiO$  phase, when used with, for example, a polyester-based magnetic tape, exhibited a friction coefficient much smaller than did conventional metal guides as will be discussed later. Not only that, but also the ceramic guides of the present invention shown hardly any fluctuation in the tension of the running tape throughout the continued use for an extended period of time. Also, the electro-conductive ceramic guides of the present invention were incorporated in high-grade tape recorders, and the amount of wow-flutter was determined according to the test tape reproducing method. The result was that the value of the determined amount was 0.02 rms or less at the tape speed of 19 cm/s. This value was about one-fifth of the value obtained by the use of a conventional metal guide. Thus, it was possible to improve the quality of tape recorders.

The reasons why the electro-conductive ceramic guide consisting of a molded sintered piece of  $TiO$  phase has a small friction coefficient and is stable against the change in ambient temperature and ambient relative humidity as stated above are considered to be explained as follows. The sintered piece of  $TiO$  phase has a crystal structure which is face-centered cubic and in addition this piece is an oxide of titanium. Therefore it has a large yield point pressure. Besides, in the crystal particles which constitute the sintered piece of  $TiO$  phase, there are present regularly disposed oxygen atoms and lattice defect of titanium. Thus, this guide has a reduced area in which it contacts the running tape or like article. And along with this, the guide has a large electro-conductivity. Accordingly, the guide does not develop any phenomenon of adhering to the tape which would be caused if the latter stores static charge. Moreover, the sintered piece of  $TiO$  phase is relatively irregular in the dispositional arrangement of the crystal particles and the non-crystal regions, and its crystal particles which are needle-like particles of a size of the order of 5-20 microns are scattered. Thus, this sintered piece of  $TiO$  phase essentially has the characteristic of being small in friction resistance.

In FIG. 3 is shown the result of determination of changes in the friction coefficient  $\mu$  when the guides of the present invention and the prior art are brought into contact with the base face of a running tape while changing the value of the load L of the running tape

under the conditions that the ambient temperature is 25° C and the ambient relative humidity is 73 percent. In the chart of FIG. 3, the vertical axis represents the friction coefficient  $\mu$ , and the horizontal axis represents the load L (gram) of the running tape. The Curve 13 indicates the change caused by the use of the electro-conductive ceramic guides A and B of the present invention. The Curve 14 indicates the change caused by the use of conventional metal guides. As will be understood from the chart of FIG. 3, the friction coefficient  $\mu$  due to the use of the ceramic guide of the present invention is of the order of 0.2. The friction coefficient  $\mu$  has a negative characteristic that the value decreases somewhat with an increase in the load L of the running tape. Nevertheless, the friction coefficient may be termed roughly as constant and has a low friction coefficient characteristic. Therefore, the guide obtained according to the present invention is suitable particularly when it is provided in a tapered configuration B as shown in FIG. 2, as compared with a conventional metal guide which has problems when it is provided in a tapered form.

In FIG. 4 is shown the result of the test on the changes in the friction coefficient of the guides of the present invention and the prior art relative to the change in the temperature at the tape speed of 19 cm/s. In FIG. 4, the vertical axis represents friction coefficient  $\mu$  and the horizontal axis represents temperature  $t$  (°C). The Curve 15 indicates the change due to the use of the electro-conductive ceramic guides according to the present invention. The Curve 16 indicates the change due to the use of the conventional metal guides. As will be understood from FIG. 4, according to the use of the guides of the present invention, a low and generally stable friction coefficient characteristic of about 0.2 is noted.

In FIG. 5 is shown the result of the test on the change in the friction coefficient of guides against the change in the relative humidity, when the tape used is a magnetic tape made of  $Co-Fe_2O_3$  and when the tape speed is 19 cm/s and when the temperature (room temperature) is 40° C. In FIG. 5, the vertical axis represents friction coefficient  $\mu$  and the horizontal axis represents relative humidity H(percent). The Curve 17 indicates the change due to the use of the electro-conductive ceramic guides of the present invention, and the Curve 18 indicates the change due to the use of conventional metal guides. As will be understood from FIG. 5, the guides according to the present invention show the change in the friction coefficient  $\mu$  the value of which is of the order of 0.2 and show a positive characteristic, i.e., the value of  $\mu$  increases somewhat with an increase in the relative humidity. However, when compared with the change due to the use of conventional metal guides, it may be said that the amount of the change is very small.

Also, tests were conducted on the hardness of the electro-conductive ceramic guides of the present invention. By Vickers hardness test with a test load of 25 grams, the hardness of the guides was found to be 1,450 - 1,600. In other words, the guides of the present invention were found to be good in workability such as cutting and grinding.

The electro-conductive ceramic guides which are each comprised of a shaped sintered piece of  $TiO$  phase have a further advantage that they are useful in inhibiting the static charging on the magnetic tapes because

of the fact that although the sintered piece of  $\text{TiO}$  phase is a metal oxide porcelain, it has a very high electro-conductivity. More specifically, the sintered piece of  $\text{TiO}$  phase is of a high electro-conductivity of the order of  $1,000 - 2,000 (\Omega - \text{cm})^{-1}$  at room temperature due to the presence of oxygen and due to the lattice defects of titanium. Therefore, even when there occurs a static charge on the magnetic tape for any reason, this static charge on the tape can be removed by being led to the outside of the system through a metal member such as a screw 2 or a threaded rod 7 as the tape is brought into contact with the guide A or B which is made with a highly electro-conductive, shaped sintered piece of  $\text{TiO}$  phase. As a result, it is possible to prevent the occurrence of an erroneous action caused by the static charging on the magnetic tape and the occurrence of wow or flutter, at the time of recording and reproduction. Moreover, the guide minimizes the deposition of dust thereon and on the tape. Thus, the guide of the present invention has much superior functions when compared with those of the guide made with an electrically insulated metal oxide porcelain.

Also, the electro-conductive ceramic guide according to the present invention is of a good thermal conductivity. Thus, it develops a very little thermal shock, and does not become over-heated during use. Accordingly, it is suitable also as a guide for use in the manufacturing process of synthetic filaments, fibers and films. In such a case, the guide serves to prevent the development of fluff of filaments, fibers and films and to prevent their sticking or adherency due to damage or generated static electricity, and thus serves to an improvement of the quality and productivity of such articles.

Next, with respect to the manufacturing method of the electro-conductive ceramic guide, metallic titanium is first mixed with titanium dioxide ( $\text{TiO}_2$ ) at the mol ratio of  $1 : 0.66 - 1.22$ , and the mixture is molded into an element of the desired shape such as A or B. This element is then sintered at a temperature of  $1,200^\circ - 1,450^\circ \text{C}$  in vacuum or in an inert gas. Thus, the sintered element is obtained as a sintered piece of  $\text{TiO}$  phase. The resulting  $\text{TiO}$  will have a composition ratio between  $\text{TiO}_{0.8}$  and  $\text{TiO}_{1.1}$  and the crystal particles of this element gains a face-centered cubic structure, which is very convenient in satisfying the objects of the present invention. More specifically, in case the mixing proportion is such that titanium dioxide is less than 0.66 relative to 1 of metallic titanium, the resulting crystal particles will have a structure which is mainly not of face-centered cubic of  $\text{TiO}$  phase, but will be that of multi-component system containing body-centered cubic or the like. This latter structure is physically fragile and accordingly is no longer proper for a guide. On the contrary, if the proportion of titanium dioxide is in excess of 1.22 relative to 1 of metallic titanium, the crystal particles will have a structure which is mainly not that of a face-centered cubic, but will be that of a multi-component system containing rhombic system or the like other than the  $\text{TiO}$  phase, which is low in electro-conductivity and physically fragile and has a large frictional coefficient and is no longer suit-

able for a guide. According to the present invention, sintering is performed in vacuum or in an inert gas, and the element is not exposed to the effect of oxygen contained in the outside atmosphere. It is, therefore, possible to obtain, accurately and easily, the desired  $\text{TiO}$  in accordance with the mol ratio between the metallic titanium and the titanium oxide. In addition, in the manufacture of the electro-conductive ceramic guide of the present invention, if it is arranged so that only that portions of the element which are brought into contact with the running tape or like article are made with such a sintered piece of  $\text{TiO}$  phase as stated above, and that the remaining portions are made with an ordinary metal material and that these two groups of portions are united to each other, it will be reasonable with respect to both the cost and the manufacturing techniques. It should be noted also that although the composition of the aforesaid  $\text{TiO}$  phase sintered piece is of the  $\text{TiO}$  ratio between  $\text{TiO}_{0.8}$  and  $\text{TiO}_{1.1}$ , the composition ratio of  $\text{TiO}_{1.0}$  is the most proper for a guide.

As stated above, the electro-conductive guide of the present invention which is comprised of a molded sintered piece of titanium monoxide whose crystal particles have a face-centered cubic crystal structure is formed with a material which is completely different from the materials of the conventional guides. The guide of the present invention is thus of a very small coefficient of friction and is capable of imparting a stable low tension continuously for an extended period of time. Besides, this guide is of a high electro-conductivity and, accordingly, it has the function of removing the static charge accumulated on the running tape or like article. Thus, the guide of the present invention can exhibit a marked effect as a guide for video tapes which require highly dense and high quality recorded sounds and recorded images.

I claim:

1. An electro-conductive ceramic guide made with a molded sintered element of titanium monoxide having portions which are brought into contact with a running tape or like article, said portions having crystal particles each consisting of a face-centered cubic crystal structure.
2. An electro-conductive ceramic guide according to claim 1, in which said portions comprises a straight body portion having an even external diameter throughout its length and a longitudinal central bore for the insertion of a screw, and a bottom plate connected to said body portion and provided with a central through-hole aligned with said bore.
3. An electro-conductive ceramic guide according to claim 1, in which said portions comprises a tapered body portion having a decreasing external diameter from base to top and a longitudinal central bore for the insertion of a threaded rod, a top plate connected to the upper end of said body portion and provided with a central through-hole for threadable engagement with said bore, and a bottom plate connected to said body portion and provided with a through-hole aligned with said bore.

\* \* \* \* \*